

June 18, 1957

J. J. STOKES, JR

2,796,456

PRIMARY CELL ANODE

Filed Feb. 8, 1955

Fig. 1.



Fig. 2.



INVENTOR  
*John J. Stokes, Jr.*  
BY *George B. Todd*  
ATTORNEY

# United States Patent Office

2,796,456

Patented June 18, 1957

1

2,796,456

## PRIMARY CELL ANODE

John J. Stokes, Jr., Unity, Pa., assignor to Aluminum Company of America, Pittsburgh, Pa., a corporation of Pennsylvania

Application February 8, 1955, Serial No. 486,758

5 Claims. (Cl. 136—100)

This invention relates to primary cells of the "dry" type and more particularly to an aluminous metal anode which also serves as the container for the cell. The term "aluminous metal" as used herein refers to both aluminum and those alloys which contain more than 50% of that element.

One of the general objects of the invention is to provide an aluminous metal dry cell container which has a longer shelf life than has been obtained heretofore with aluminum containers. Another object is to provide a container or can which offers an improved cell performance without perforation of the container wall. Still another object is to provide a dry cell container of composite construction in which the base or supporting component closely resembles the anode alloy in electrical characteristics and hence if the anode is consumed or fails, the supporting member can serve as the anodic component of the cell. A particular object is to provide a duplex aluminous metal dry cell container which permits substantially complete consumption of the anode without perforation of the container wall. Other objects will be apparent in the following disclosure and from the drawings wherein.

Fig. 1 is a somewhat diagrammatic view partly in section illustrating a dry cell structure embodying the invention, and

Fig. 2 is an enlarged sectional view of a portion of the container wall illustrating its composite construction.

Primary cells having aluminum anodes have been proposed heretofore in order to take advantages of the relatively high electrochemical equivalent of aluminum as compared to that of zinc, the metal extensively employed heretofore in the construction of dry cells. Such cells containing aluminum anodes, however, have suffered from at least two drawbacks, namely, the accumulation of oxide film on the anode, especially if the cell is kept on the shelf for extended periods of time, which interferes with quick response for current when placed in a circuit, and perforation of the cell wall either during service or during storage if the common halides are used as the electrolyte. My invention is directed to overcoming these disadvantages and to using aluminous metal in a more efficient manner.

My invention broadly comprises the discovery that an improved dry cell can be made by forming the container or shell from a composite aluminous metal body wherein the inner portion in contact with the electrolyte consists of a special aluminum base alloy and the second or outer portion is composed of aluminous metal of a different composition which has a lower electrode potential, i. e. it is less anodic toward the cathode than the inner layer. For operation of the cell it is of course necessary to use an electrolyte which is adapted to serve in contact with aluminum and aluminum base alloys. The special anode alloy which I have found to be superior to other aluminum base alloys not only gives a high output in closed circuit but permits storage in open circuit condition without substantial loss in efficiency. The outer or supporting alloy

2

layer although slightly less efficient than the anode alloy can readily serve as the anode without any significant change in the potential of the current supplied by the cell.

5 Various electrolytes, especially solutions, have been suggested for use in contact with aluminum anodes but I have found that superior results are obtained by employing aluminum chloride hexahydrate and ammonium, sodium or potassium chromate in the cell paste in combination with manganese dioxide and finely divided carbon. The improved electrolyte forms the subject matter of my co-pending application Serial No. 486,757, filed on even date herewith.

Although aluminum can be used as the anode of a primary cell if the above mentioned electrolyte is employed, I have found that much better performance is obtained over a longer period of time if the anode consists of an alloy composed essentially of aluminum and at least one alloying component of the group consisting of 15 0.001 to 5% zinc, 0.02 to 0.5% tin, 0.02 to 1% bismuth, 0.1 to 10% magnesium and 0.5 to 2% of the intermetallic compound Mg<sub>2</sub>Si. Minor amounts of other elements such as boron, titanium, chromium and manganese may also be present in quantities usually employed in aluminum base alloys to impart some desired property to the alloy. Under some circumstances it may even be desirable to include a small amount of copper, less than 0.5%. For the sake of convenience these alloys may be referred to as anode alloys. A container made of one of these 20 alloys is substantially uniformly attacked over the entire inner surface by the electrolyte in the cell and does not acquire a film which obstructs action by the electrolyte. Moreover, these alloy additions tend to increase the electrode potential of the anode which, of course, is advantageous. Of the various alloys I prefer the aluminum-zinc composition and for optimum results an alloy of aluminum of a purity of not less than 99.8% and from 0.5 to 1.5% zinc is preferred.

While the several alloys mentioned above serve very well as a consumable anode shell or container from the standpoint of current output, they suffer from the disadvantage of being perforated if there is severe local attack. To overcome this disadvantage and yet derive the desired benefits from the alloys, an outer layer or 40 sheath of aluminous metal of a different composition is provided which has a lower electrode potential than the inner layer. Generally, this difference should amount to at least 0.1 millivolt and should be within the range of 0.1 to 200 millivolts. Greater differences cause excessive 45 consumption of the anode alloy. The alloys used for the outer layer must be chosen with respect to the electrode potential of the inner layer. The electrode potential of a given alloy can be determined according to standard methods, for example, by use of a calomel half cell and 50 solution of the electrolyte to be used in the cell. Suitable alloys for the outer layer are such well known ones as the aluminum-manganese and aluminum-magnesium silicide types. In addition, commercially pure aluminum of 99.2% purity, and even aluminum of lower purity can 55 be used for the outer layer. Alloys which can be readily worked and formed into containers are preferred. An alloy which is preferred for the shell is one composed of aluminum and from 0.5 to 1.5% manganese.

The composite aluminous metal container of my invention 60 consists of a relatively thick inner layer of the anode alloy and a relatively thin outer layer of the less anodic metal. In general, the anode composition should constitute as large a proportion, not less than half, of the total thickness of the shell wall as is practicable, usually 65 within the range of 50 to 90% of the total thickness. According to my preferred practice the inner layer should 70

constitute from 60 to 80% of the total thickness of the composite shell.

In operation of the cell the anode alloy is gradually consumed and when any pits develop which extend through the inner alloy layer and reach the outer layer they become enlarged by spreading laterally rather than perforating the remainder of the container wall. This behavior of the inner layer is brought about by creating and maintaining a difference in electrode potential between the two components, the inner alloy layer having the higher potential. If the cell is kept in service until the anode alloy has largely disappeared, the cell can still deliver substantially the same current for a short period of time. In this respect, my composite shell differs from any duplex cell containers which have been proposed heretofore. It also means that the maximum output of the cell is obtained over a longer period of time because perforation of the shell does not occur until a major portion of the anode has been consumed.

The composite shell or container should have a wall thickness equivalent to that employed in the dry cell art where zinc is used. For small cells such as used in flashlights, the shell may be from 0.010 to 0.015 inch in thickness whereas in larger shells, such as the common No. 6 size, the wall may be 0.018 to 0.020 inch in thickness. Of course, a heavier shell may be employed but this must be balanced against the amount of electrolyte present in the paste mixture.

The composite material from which the container or shell is formed may be fabricated in any conventional manner. For example, sheets or slabs of the two alloys may be bonded together by hot rolling, or one alloy may be cast against a slab of the other one and the resulting body hot rolled. Still another method is that of spraying the anode alloy upon the outer or supporting layer. Still another method of fabrication is that of producing the containers or cups from composite slugs by the impact extrusion process. The forming of the containers from sheet products may be accomplished in conventional manner such as by drawing. In all cases it is important that the anode alloy be firmly bonded to the supporting member and thereby avoid any separation or scaling during the operation of the cell.

Referring to Fig. 1 which illustrates one embodiment of my invention, it will be seen that a composite cylindrical shell 1 consisting of an inner anode layer 2 and an outer layer 3 is lined with an inert absorbent paper 4, the top edge of which is crimped inwardly to assist in retaining the paste in position. The paper layer serves to prevent direct contact of the mix with the shell yet is permeable to the electrolyte. A conventional carbon rod 5 centrally disposed in the shell is the cathode. Between the paper lined shell and the carbon rod is the paste 6 containing the electrolyte, depolarizer and finely divided carbon. Above the paste is a space 7 which can accommodate any expansion of the paste that may occur without rupturing the cell wall or the top seal. The cell is sealed by a suitable plastic or resinous substance 8 in association with a fibrous separator 9. The carbon rod 5 is provided with a conventional metal cap 10 to insure good electrical contact with another metallic conductor.

In the enlarged view of a portion of the cell wall shown in Fig. 2, the duplex character of the aluminous metal container wall is plainly evident. The inner layer 2 of the anode alloy is much thicker than the outer layer 3. The paper liner 4 in contact with the inner layer 2 and the electrolyte paste 6 are also shown.

For many purposes it is desirable to provide a paper or other insulative cover for the cell. Such covers are well known and need not be described.

It will be appreciated that the primary cells which may employ the composite shell described above may vary considerably in size. The composite shell has been found to be especially useful for the production of small cells of the type used in flashlights and similar articles.

The improvement gained from the use of a composite shell as compared to a shell of a single composition is illustrated in the following example. Flashlight cells were made which were identical except as to the composition of the shells. Each cell had a carbon rod cathode and an electrolyte paste composed of aluminum chloride hexahydrate and potassium chromate in equal parts, manganese dioxide, carbon black and water. The shell in one case consisted of aluminum of 99.8% purity and the other shell was of the composite type, the inner layer constituting 70% of the total thickness of the shell wall and composed of an aluminum-zinc alloy made from 1% zinc and aluminum of 99.8% purity, and the outer layer composed of an aluminum base alloy consisting of aluminum and 1.25% manganese, the two layers having been bonded by hot rolling them together. In a shelf life test the first type of cell exhibited perforation of the shell in eight months whereas no failure occurred in the second type after a fourteen month storage.

Having thus described my invention and an embodiment thereof, I claim:

1. A primary cell of the dry type comprising a cathode, an electrolyte and a composite aluminous metal container as the anode, said container consisting of two metallic layers of different composition, the inner layer in contact with the electrolyte constituting more than half the total wall thickness of the shell, said inner layer also consisting of an alloy composed essentially of aluminum and at least one alloying component selected from the group consisting of 0.001 to 5% zinc, 0.02 to 0.5% tin, 0.02 to 1% bismuth, 0.1 to 10% magnesium and 0.5 to 2% of the intermetallic compound  $Mg_2Si$ , and the outer layer composed of aluminous metal having an electrode potential below that of the inner alloy layer, said layers being firmly bonded together.

2. A primary cell of the dry type comprising a cathode, an electrolyte and a composite aluminous metal container as the anode, said container consisting of two metallic layers of different composition, the inner layer in contact with the electrolyte constituting from 50 to 90% of the total wall thickness of the shell, said inner layer also consisting of an alloy composed essentially of aluminum and at least one alloying component selected from the group consisting of 0.001 to 5% zinc, 0.02 to 0.5% tin, 0.02 to 1% bismuth, 0.1 to 10% magnesium and 0.5 to 2% of the intermetallic compound  $Mg_2Si$ , and the outer layer composed of aluminous metal having an electrode potential at least 0.1 millivolt below that of the anode alloy of the inner layer, said layers being firmly bonded together.

3. A primary cell of the dry type comprising a cathode, an electrolyte and a composite aluminous metal container as the anode, said container consisting of two metallic layers of different composition, the inner layer in contact with the electrolyte constituting from 50 to 90% of the total wall thickness of the shell, said inner layer also consisting of an aluminum-zinc alloy composed of 0.001 to 5% zinc and aluminum of a purity not less than 99.8%, and the outer layer composed of an aluminous metal having an electrode potential at least 0.1 millivolt below that of the aluminum-zinc alloy, said layers being firmly bonded together.

4. A primary cell of the dry type comprising a cathode, an electrolyte and a composite aluminous metal container as the anode, said container consisting of two metallic layers of different composition, the inner layer in contact with the electrolyte constituting not less than half the total wall thickness of the shell, said inner layer also consisting of an aluminum-zinc alloy composed of 0.5 to 1.5% zinc and aluminum of a purity not less than 99.8%, and the outer layer composed of an aluminum base alloy consisting of aluminum and 0.5 to 1.5% manganese, said layers being firmly bonded together.

5. A primary cell of the dry type comprising a cathode, an electrolyte and a composite aluminous metal container

as the anode, said container consisting of two metallic layers of different composition, the inner layer in contact with the electrolyte constituting from 60 to 80% of the total wall thickness of the shell, said inner layer also consisting of an aluminum-zinc alloy composed of 0.5 to 1.5% zinc and aluminum of a purity not less than 99.8%, and the outer layer composed of an aluminous metal having an electrode potential below that of the aluminum-zinc alloy, said layers being firmly bonded together.

## References Cited in the file of this patent

## UNITED STATES PATENTS

|           |            |       |               |
|-----------|------------|-------|---------------|
| 2,199,445 | Ruben      | ----- | May 7, 1940   |
| 2,554,447 | Sargent    | ----- | Jan. 26, 1949 |
| 2,712,564 | Fry et al. | ----- | July 5, 1955  |